

## UNITED STATES PATENT OFFICE

AXEL WILLIAM NÖRLANDER, OF STOCKHOLM, SWEDEN, ASSIGNOR TO AKTIEBOLAGET  
RAPIDOGRAFI, OF STOCKHOLM, SWEDEN, A COMPANY OF SWEDEN

## METHODS OF PRODUCING PRINTING PLATES OR THE LIKE

No Drawing. Application filed March 7, 1928, Serial No. 259,920, and in Sweden March 18, 1927.

The present invention relates to a method of producing printing plates or the like which may be used for direct printing, and more especially to the production by the action of light of printing plates from supported or non-supported layers or films containing one or several silver salts. The invention is characterized principally by the fact that the layer or film prior to exposure is treated with one or several hardening agents such as alum, formaline, chrome alum and so forth. The hardened layer is then treated with a solution of one or several light-sensitive chromium salts, exposed to the action of light and subjected to an after-treatment with acid or acids, when the layer, for instance by being moistened and treated with a fat dye or ink, may immediately be used either for direct printing or for transfer of the image, for instance upon zinc and subsequent treatment in known manner.

This method of producing printing plates or the like, which will be more fully described in the following specification, offers considerable advantages in many respects over the methods heretofore used in the art.

The plates produced according to the invention, it being understood that the word plate is used in the following to denote the supported as well as the non-supported layer or film, are characterized by greater light-sensitivity as compared with the plates or the like used in other similar processes, and consequently a considerably shorter time of exposure may be used. The reproduction on the plate of the image to be printed may be effected in known manner by direct printing from a negative—in some cases a positive,—or by direct exposure as in a camera, but such reproduction may also, as distinct from the methods heretofore in use in the art of reproduction, be effected without difficulty while the image is simultaneously being enlarged, for instance by projection, which is of great advantage. Heretofore, such projection could not be practically carried out with any reasonable degree of enlargement, owing to the very long time of exposure required therefor. Thus, if an enlargement was to be produced according to any of the known meth-

ods, it was necessary first of all to produce a negative of the same or about the same size as the desired printing plate, which represented a good deal of expense and loss of time. According to the present invention, however, an enlargement may be made direct by projection and in a comparatively short period of time. 55

Another advantage which is characteristic of the method according to the present invention, is that the exposed and after-treated plate may be used immediately for direct printing, and that a very great number of prints may be taken from the same plate without perceptible falling off of the quality 60 of the printed image. The image may also be transferred upon zinc in the usual way, for example for etching. 65

By a special procedure, which also forms an object of the invention, the sensitive layer 70 may be mounted on the support, when such a support is being used, by means of an intermediate layer, which considerably increases the cohesion between the sensitive layer and the support. As a result of this powerful 75 cohesion such a material as for example a zinc-plate may be used as the support and the finished printing plate may be bent to be used for example for off-set printing without the layer working loose from the support. 80

The method is suitable not only for the production of printing plates capable of reproducing the lights and shadows of the original, but is also, by certain modifications, 85 suited for production of so-called high and deep print stereotypes and screens.

The prints are distinguished by the exceedingly accurate reproduction of the details of the original as well as of the lights 90 and shadows thereof.

The method will now be described in detail by way of an example, but many modifications will be apparent to those skilled in the art without departing therefrom or from 95 the scope of the claims.

If a support or base is to be used, which may consist of any suitable material, such as glass, zinc, nickel, metal etc., the support is preferably prepared for the application of the 100

sensitive layer, in the following manner. The support is carefully cleaned, for instance with hot water, and is then coated with a solution of gelatine containing large quantities 5 of water-glass, for instance one part of water-glass and five parts of saturated gelatine. The mixture is preferably prepared at a temperature of 50-60 degrees centigrade and must, when applied to the support, be kept 10 warm as well as the latter. After cooling the support is ready to receive the sensitive layer.

This sensitive layer, which preferably consists of a silver salt-gelatine emulsion, may be prepared in the following manner. 100 15 grams of gelatine are placed in cold water for one hour, the excess of water is drained off and the saturated gelatine heated. When melted 10 grams of silver nitrate are added together with an equivalent quantity of sodium chloride and the mixture is boiled for 20 25 5 to 10 minutes, while being stirred, in non-actinic light, whereupon it is permitted to cool, when it will solidify. For washing out any excess of salts, the solidified mass is finely divided and washed in running water for about 12 hours. This stock mixture will keep in a dark room.

When used, one part of the stock mixture is boiled with two parts of gelatine saturated 30 with water in non-actinic light during a period of about 5 minutes. The mixture is permitted to cool to about 40 degrees centigrade, when it is poured out on the prepared supports, which are then allowed to dry. By 35 dilution or concentration of the silver salt-gelatine mixture and by controlling the temperature at which the coating of the supports takes place, the thickness of the layer and thus, to a certain extent, the printing effect 40 thereof, may be varied at will.

When dry, the layer is hardened in a solution of alum, formaline, chrome alum or the like. A suitable bath for this purpose consists of a saturated solution of alum in 45 water. In this bath the silver salt-gelatine layer is hardened for about 5 minutes, whereupon the plates are washed and dried. Plates produced in this manner will keep in a dark room.

50 The hardening may also be carried out by first subjecting the layer to a pre-hardening with alum and then to an after-hardening with formaline, for instance one part of formaline to 25-40 parts of water. In this way 55 a harder layer is obtained.

To prevent the gelatine layer from working loose from the support during the after-treatment, the edges of the layer are preferably coated with a solution of shellac.

60 If a printing plate is to be produced from these stock plates, the gelatine layer is bathed in an 8% solution of ammonium bichromate admixed with ammonia until the solution has assumed a light yellow colour— 5 one part of ammonia to ten parts of bichro-

mate solution. The plate is dried at a temperature of 40-45 degrees centigrade, which requires a time of about two hours, more or less, depending on the thickness of the gelatine layer, and is then ready to take up the 70 desired image by exposure, which may take place in different ways, as stated hereinbefore, *inter alia* also by projection under simultaneous enlargement of the image. The importance of this has already been pointed out, and as an example of the short periods of exposure which can be employed, it may be mentioned that the time of exposure for making a stereotype of the dimensions 20-26 centimeters from a negative 9-12 centimeters, using a 30 ampere arc lamp, is about 5 80 minutes only. With regard to the source of light, it should of course be observed, that in order to obtain as short an exposure as possible, the source of light should give off a sufficient quantity of actinic or short-wave light.

85 In certain cases it may be preferable to undertake a hardening also after the exposure.

90 The exposed plate is then subjected to an after-treatment with acids. A suitable solution for this purpose may consist of 1 part of sulphuric acid and 15 parts of water; the time of treatment is generally 1-2 minutes 95 depending on the time of exposure and other circumstances.

100 It is of importance that the edges of the gelatine layer are coated with shellac prior to the after-treatment in order to prevent liquid from entering the space between the layer and the support and thus separating them. The printing plate may be used immediately for printing in a press, for instance by being moistened and treated with 105 fat dye or colouring matter, or the image may be transferred in known manner for instance upon zinc for etching.

110 For the production of screens the sensitive layer is exposed directly in evenly distributed or diffused light, a stipple or grain structure being then obtained after the acid treatment, said structure having requisite screening effect. It is also possible, however, to expose through one of the screens used in the 115 art of reproduction, the procedure otherwise being the same as described.

120 Deep-print stereotypes may be produced by exposing through a negative and treating the surface, subsequent to after-treatment and moistening, with fat colouring matter, whereupon the plate is dried.

125 High-print stereotypes may be produced in a similar manner, with the difference only that the plate is exposed to the action of light through a positive.

130 The whole process as hereinbefore described represents a great saving of time, inasmuch as finished stereotypes having the same size as the original picture or layer

or smaller may be produced in a few hours or even in a shorter time from the stock plates.

What I claim is:—

5 1. The process of making a printing plate which can be used for direct printing, comprising incorporating in a colloid film a silver halid, hardening the film, treating the hardened film with an alkali bichromate, exposing the film to the action of light and selectively modifying the hardening with an agent of suitable pH-concentration.

10 2. A process as defined in claim 1 in which the silver halid is silver chloride.

15 3. A process as defined in claim 1 in which the hardening agent is alum.

4. A process as defined in claim 1 in which the silver halid is silver chloride and the hardening agent is alum.

20 5. A process as defined in claim 1 in which the alkali bichromate is used in the form of a solution of ammonium-bichromate admixed with ammonia.

6. The process of making a printing plate 25 which can be used for direct printing, comprising incorporating in a colloid film silver chloride, hardening the film with alum, treating the hardened film with a solution of ammonium bichromate admixed with ammonia, exposing to the action of light and selectively modifying the hardening with an agent of suitable pH-concentration.

30 7. A process as defined in claim 1 in which the agent employed for modifying the hardening is an acid.

35 8. A process as defined in claim 6 in which the agent employed for modifying the hardening is an acid.

9. A process as defined in claim 6 in which 40 the agent employed for modifying the hardening is diluted sulfuric acid.

10. The process of making a printing plate 45 which can be used for direct printing, comprising incorporating silver chloride in gelatine, hardening the gelatine with alum, treating the hardened gelatine with a solution of ammonium bichromate admixed with ammonia, exposing to the action of light and selectively modifying the hardening with diluted sulfuric acid.

50 11. The process of making a printing plate which can be used for direct printing, comprising incorporating a silver halid in gelatine, hardening the gelatine with a hardening 55 agent, treating the hardened gelatine with a solution of an alkali bichromate, exposing to the action of light while enlarging and modifying the hardening with an acid.

12. The process of making a printing plate 60 which can be used for direct printing comprising incorporating a silver halid in gelatine, hardening the gelatine with a hardening agent, treating the hardened gelatine with a solution of an alkali bichromate, exposing to the action of light, hardening again

and selectively modifying the hardening with an acid.

13. The process of making a stereotype 70 which can be used for direct printing, comprising incorporating a silver halid and an alkali bichromate in a colloid film, exposing to the action of light, selectively modifying the hardening with an agent of suitable pH-concentration, moistening and rolling over the treated surface with dye and drying.

14. A process of making a stereotype 75 which can be used for direct printing comprising incorporating silver chloride in gelatine, hardening the gelatine with alum, treating the hardened film with a solution of ammonium bichromate admixed with ammonia, exposing to the action of light, selectively modifying the hardening with sulfuric acid, moistening and rolling over the treated surface with dye and drying.

15. A sensitized plate to be used for making a printing plate comprising a hardened colloid film in which is incorporated a silver halid and an alkali bichromate.

16. A sensitized plate to be used for making a printing plate comprising a hardened gelatine film in which is incorporated silver chloride and ammonium bichromate.

In testimony whereof I affix my signature.

AXEL WILLIAM NORDLANDER.

70

75

80

85

90

95

100

105

110

115

120

125

130